

United States Patent [19]  
Greenstein

[11] 3,865,742  
[45] Feb. 11, 1975

[54] RESISTOR COMPOSITIONS

[75] Inventor: **Bernard Greenstein**, Toledo, Ohio

[73] Assignee: **Owens-Illinois, Inc.**, Toledo, Ohio

[22] Filed: **May 6, 1971**

[21] Appl. No.: **140,988**

[52] U.S. Cl..... **252/63.5**, **252/514**, **29/610**,  
29/620, 338/224, 338/226, 106/53, 106/54,

117/23, 117/160 R, 117/169 R, 117/169 A, 117/227

[51] Int. Cl.... **H01b 3/02**, **H01h 85/24**, **H01c 17/00**

[58] Field of Search ..... **252/514**, **63.5**; **117/227**,  
117/23, 160 R, 169 R, 169 A; **106/47**, **53**, **54**

[56] References Cited

UNITED STATES PATENTS

|           |         |                       |                 |
|-----------|---------|-----------------------|-----------------|
| 3,154,503 | 10/1964 | Janakirama-Rao et al. | ..... 252/514   |
| 3,252,831 | 5/1966  | Ragan                 | ..... 117/227 X |
| 3,407,081 | 10/1968 | Ballard               | ..... 252/514 X |
| 3,516,857 | 6/1970  | Short                 | ..... 117/227 X |
| 3,537,892 | 11/1970 | Milkovich et al.      | ..... 117/227   |

|           |        |              |               |
|-----------|--------|--------------|---------------|
| 3,634,334 | 1/1972 | Burgess      | ..... 252/514 |
| 3,681,261 | 8/1972 | Mason et al. | ..... 252/514 |
| 3,717,453 | 2/1973 | Daiga        | ..... 75/5 A  |

FOREIGN PATENTS OR APPLICATIONS

|           |        |               |               |
|-----------|--------|---------------|---------------|
| 1,026,577 | 4/1966 | Great Britain | ..... 252/514 |
|-----------|--------|---------------|---------------|

Primary Examiner—**Roland E. Martin, Jr.**  
Attorney, Agent, or Firm—**Richard B. Dence; E. J.**  
**Holler**

[57] ABSTRACT

A printed microelectronic resistor having excellent stability, high reproducibility and a TCR less than about  $\pm 500$  ppm/ $^{\circ}$ C (25°–150° $^{\circ}$ C) is formed from a composition comprised of a glass binder and a silver chloride or cyanide salt free, homogeneous, finely divided powdered admixture of a resistive metal, silver and gold, the powder having a particle size of less than about 5 microns.

26 Claims, No Drawings

## RESISTOR COMPOSITIONS

This application relates to electronic resistors and methods of making same. More particularly, this invention relates to electronic resistors, compositions, pastes, and methods of making and using same, particularly within the environment of microelectronic circuitry.

As explained in commonly owned copending application Ser. No. 58,740 filed July 27, 1970, now U.S. Pat. No. 3,681,261, the art has long known of the value of palladium oxide (PdO) for use as a resistor material, particularly in microelectronic circuitry. Generally speaking, palladium oxide is formed into a resistor by admixing palladium with a glass binder and organic vehicle to form a printing paste. In the case of microelectronic circuitry, the paste is then printed onto a dielectric substrate such as aluminum oxide or the like by the use of a screen or mask of the desired mesh and formed to provide the desired pattern. The patterned design is then fired in air to oxidize the Pd to PdO and form the ultimate resistor lamina.

In order to increase the negative temperature coefficient of resistivity (hereinafter referred to as TCR), to regulate ultimate resistivity, and to render the stability of the PdO system acceptable, certain metals are employed in admixture with the palladium in the paste. Such metals, which are referred to hereinafter as stabilizers, are those which do not oxidize at the temperatures used to fire the printed paste.

Many problems attend these prior art PdO resistor systems. One major problem is the great sensitivity of these systems to the firing process as a whole. Slight fluctuations or variations in the firing temperature, for example, greatly change the resistivity of the resulting product. Air flow and firing times are further variables to which the ultimate characteristics of the final product are extremely sensitive. Such sensitivity, of course, renders these PdO systems extremely difficult to reproduce. Not only is reproducibility low, but for some reason, not entirely understood, stability is also very low.

The term "stability" is well-understood in the art and is used herein in accordance with this well-known meaning. This is to say, stability defines that characteristic of a resistor which enables it to maintain its resistivity within tolerable limits over extended periods of time and use.

While the stabilizer metals used in admixture with the palladium oxide generally provide commercially tolerable stability to the system, they are generally found to detrimentally increase the TCR of the systems, usually far above the  $\pm 0$  ppm/ $^{\circ}\text{C}$  level ideally desired. In some instances, especially when Ag is used, stability must be sacrificed for acceptable TCR while, on the other hand, TCR must be sacrificed for acceptable stability. In almost all instances, reproducibility, regardless of the metal stabilizers used, is detrimentally low.

In order to overcome these problems, the art has sought out many solutions. Some have sought to use various additional additives to improve the system. Others have sought to alter the starting materials employed such as by employing finely divided palladium oxide in the paste or initially employing crystalline palladium or its oxide within critical particle sizes and surface areas. Others used combinations of the above solutions or turned completely from the PdO system to seek other resistive metal oxide systems which might have higher stability and/or reproducibility. In many in-

stances, only a modicum of success was actually achieved. In many other instances, the manufacture was rendered so expensive as to make it economically undesirable.

5 In fulfillment of the need arising out of the above-described problems, commonly owned copending application Ser. No. 58,740 filed July 27, 1970, now U.S. Pat. No. 3,681,261 provides the art with a valuable technique for forming resistive metal oxide systems of the PdO type which are highly stable, reproducible, and have excellent TCR values. The entire disclosure of this last-mentioned patent is incorporated herein by reference.

Generally speaking the resistor compositions are 15 formed in accordance with this last-mentioned patent by:

- a. forming an admixture of a resistive metal-organometallic compound, at least one metal stabilizer in organometallic form and an anti-agglomerating agent 20 which will remain in the system throughout processing;
- b. heating the admixture at a sufficient temperature and for a sufficient period of time to drive off the organo-constituents and concentrate the admixture to a powder; and
- 25 c. heating the powder at a sufficient temperature and for a sufficient period of time to alloy said metals and in some instances to oxidize the resistive metal.

The powder resulting from step (b) is an admixture 30 extremely homogeneous in nature, which upon alloying in step (c) results (because of this high homogeneity) in a uniquely insensitive base material from which stable, reproducible resistors can be formed having low absolute TCR values. While only one stabilizing metal may be employed, it was found to be preferred to use 35 at least two of these metals together in amounts which were found to synergistically reduce their effect upon TCR. Thus, by using two metals in combination, excellent stability is attained without unduly increasing TCR.

40 Examples of preferred admixtures in parts-by-weight ratio for minimization of the effect upon TCR were disclosed as including Ag:Au about 4:1 - 1:4; Pt:Ag; about 8:1 - 1:8; and Pt:Au, about 8:1-1:8. Particularly preferred was the Ag:Au admixture since it was found 45 that this admixture when alloyed with Pd will form a single phase alloy, thus further minimizing the effect of firing on the system.

While the technique of U.S. Pat. No. 3,681,261 hereinabove described is extremely valuable, it has a few 50 drawbacks attendant with it which make the findings of an alternative technique for forming highly homogeneous resistive powders and an alternative technique for forming resistor compositions therefrom most desirable. Examples of such drawbacks include the relatively high expense of the organo-metallic compounds used as starting materials and the pollution and danger 55 caused by the volatilization of the organo-constituents during heating to powder form. It has also been found that many of the commercially available organometallics useful in the practice of that invention contain certain chlorinebearing solvents. During the concentration step (b), the chlorine ions have a tendency to react 60 with the silver metal and thereby form silver chloride precipitate which contaminates the resulting powder. 65 For the purposes of this invention wherein electronic, and more particularly microelectronic, resistors are formed, silver chloride, in any substantial amounts, can

not be tolerated in the system since it has a highly detrimental effect upon stability and the physical structure of the ultimate product.

Concurrently filed, commonly owned, copending application Ser. No. 141,006 filed May 6, 1971, now U.S. Pat. No. 3,717,453 in the name of Valdis R. Daiga and entitled POWDERS OF METAL, SILVER AND GOLD AND PROCESSES FOR MAKING SAME fulfills the above-described need of an alternative technique for forming highly homogeneous resistor powders since it eliminates the problems caused by the use of organometallics. The entire disclosure of U.S. Pat. No. 3,717,453 is incorporated herein by reference.

Generally speaking this copending application discloses two alternative techniques for forming extremely homogeneous powders of at least one other metal with silver and gold. In one technique, silver chloride or cyanide is present, albeit in reduced amounts, in the final product. Such a technique and powder formed therefrom are not contemplated for use in this invention.

The second alternative technique of U.S. Pat. No. 3,717,453 forms a non-contaminated powder which may be used as the preferred starting material for this invention. Generally speaking, this second alternative technique of this copending application, as adapted for the purposes of this invention, comprises initially forming a soluble salt solution of at least one resistive metal and silver. To this silver-resistive metal salt solution there is then added a finely divided gold powder usually having a particle size less than about 5 microns, preferably less than about 2 microns and most preferably substantially submicron in size. The solution containing the gold powder, which is not soluble in the salt solution, is then thoroughly mixed, by agitation, to form a slurry of the gold and there is then added thereto a reducing agent for the resistive metal and silver which precipitates metallic metal and silver without any substantial amount of salt being present therein. While some small amount of homogeneity is sacrificed because the gold powder is not precipitated, precipitation of the metal and silver into the slurred gold powder effects a substantial amount of homogeneity to the extent that excellent, reproducible, stable products can be made therefrom for the purposes of this invention.

The powders formed from the above-described technique, because of the soluble nature of the salt formed in solution remain uncontaminated with detrimental silver chloride or cyanide. Such powders, therefore, generally comprise a finely divided substantially homogeneous admixture of at least one resistive metal other than silver or gold, with silver and gold, which admixture is substantially free of silver chloride or cyanide. The particle size of the powder, without comminution, is generally less than about 5 microns and usually is submicron in size. Thus the powder is said to be "finely divided".

The homogeneity achieved, as stated in U.S. Pat. No. 3,717,453 is beyond that achievable by mere mechanical comminution alone or combined with single alloying and is usually to the point where the silver and resistive metal are actually alloyed together according to x-ray diffraction indications. The term "homogeneous" is therefore defined, and is so used for this invention, by this description.

While the above-described concurrently U.S. Pat. No. 3,717,453 fulfilled a first need for a preferred starting material alternative to those formed by the organo-

metallic technique, it was left to this invention to fulfill the second need of providing a resistor composition and technique alternative to those of the organometallic concept. This invention, most definitely, fulfills this second need.

Generally speaking, this invention fulfills this second need by providing the art with a resistor composition comprising a glass binder admixed with a substantially homogeneous finely divided, chloride or cyanide salt free powder comprised of at least one resistive metal and at least two stabilizer metals. Preferably, the powder also contains an antiagglomerating agent, which is substantially homogeneously dispersed throughout the powder. It is also preferred that at least one of the resistive metals be alloyed with at least one of the stabilizer metals as indicated by conventional x-ray diffraction techniques.

Generally speaking, any one or a combination of the conventional resistive metals may be used in the practice of this invention. Examples of such metals include palladium, rhodium, iridium, ruthenium, indium, and mixtures thereof. Because of the economic advantages, ease of processing, good stability, and good reproducibility, the palladium oxide system, and thus palladium, is preferred for the purposes of this invention. Examples of other metals useful in combination with silver and gold include platinum, copper, nickel and mixtures thereof.

Any of the well-known stabilizing metals may be used in the practice of this invention. Generally, these metals are chosen for their inertness to oxygen at the operating conditions of this invention. The stabilizer metal systems of this invention include at least two metals used together in amounts which have been found to synergistically minimize their effect upon TCR. Examples of these stabilizing metal systems include admixtures of silver, gold, and platinum. Examples of preferred admixtures in parts-by-weight ratio for minimization of effect on TCR include Ag:Au, about 4:1-1:4; Pt:Ag, about 8:1-1:8; and Pt:Au, about 8:1-1:8. Particularly preferred for the purposes of this invention is the Ag:Au admixture since it is found that this admixture when alloyed with Pd will form a single phase alloy, thus further minimizing the effect of firing on the system, thereby increasing reproducibility.

The anti-agglomerating agents useful for the purposes of this invention are those conventional materials which are inert to the system and which will not burn out at alloying and/or firing temperatures. Such anti-agglomerating agents are usually of a fine particle size, i.e., less than about 5 microns and usually submicron in size. Examples of these agents include: ultrafine alumina, ultrafine  $TiO_2$ , and other ultrafine refractories. Preferred for the purposes of this invention is ultrafine silica which is purchasable under the trademark CAB-O-SIL and has a submicron particle size.

This invention also envisions the use of other additives, known in the art, to the above ingredients in order to enhance, in a known fashion, one or more of the desired characteristics of the system.

Because the silver-gold stabilizer system is particularly preferred for the purposes of this invention and because the only known way to safely form a non-contaminated (free of silver chlorides or cyanides) homogeneous, finely divided powder of a resistive metal (e.g. palladium) with silver and gold is disclosed in the above-described U.S. Pat. No. 3,717,453, the tech-

nique and powders disclosed therein and incorporated herein by reference, are preferred for the purposes of this invention. This is not to say, however, that these are the only powders contemplated for use herein. Quite to the contrary, U.S. Pat. No. 3,717,453 solves a particular problem relative to silver and gold, and other noble metal combinations experiencing similar difficulties. In those instances where other stabilizer systems are employed, which systems are dissolvable in a common solution with the resistive metal without the formation of a contaminating insoluble salt of the chloride or cyanide type, simple tri-precipitation with a known reducing agent or combination of reducing agents may be effected to achieve the contemplated and necessary degree of homogeneity for the purposes of this invention. While co-precipitated powders alone or admixed with a vitreous binder are known (as exemplified by U.S. Patent No. 3,385,799 and 3,390,981 and British Patent No. 1,004,653), triprecipitated powders having a combination of two synergistically active stabilizer metals are believed to be unique to this invention.

The glass binders useful in this invention are any of the conventional glass binders employed by the art. Examples of these binders include the borosilicates and particularly the lead-alumina borosilicates. An example of such a binder includes by weight about:

|                                |        |
|--------------------------------|--------|
| SiO <sub>2</sub>               | 8-12%  |
| B <sub>2</sub> O <sub>3</sub>  | 20-30% |
| Al <sub>2</sub> O <sub>3</sub> | 2-7%   |
| ZnO                            | 20-30% |
| PbO                            | 30-40% |

A particularly preferred glass binder system for the purposes of this invention is a zinc free, boron free, lead, barium, silicate having a firing temperature (i.e. the temperature at which the glass binder flows to form a continuous binding phase for the resistor product) of about 725°-775°C and preferably about 750°-775°C. An example of these glasses includes by weight about:

| Constituent                          | Range              | Specific Example |
|--------------------------------------|--------------------|------------------|
| PbO                                  | 40-75              | 59               |
| SiO <sub>2</sub>                     | 15-40              | 31               |
| Bi <sub>2</sub> O <sub>3</sub>       | 0-15               | 2                |
| BaO                                  | 0-15               | 8                |
| Bi <sub>2</sub> O <sub>3</sub> + BaO | 2-30               | 10               |
| other oxides                         | less than about 10 | substantially 0  |

An example of ther oxides include Al<sub>2</sub>O<sub>3</sub>, CaO, ZrO<sub>2</sub> and the like. These glasses have been found to form excellent structures of high cosmetic quality when they are employed in the requisite amounts.

Many of the glass binders contemplated by this invention, such as those of the borosilicate type, do not adversely affect the absolute value of TCR in the system and may therefore be employed alone without additive adjustment. On the other hand, the TCR effect of the preferred zinc free, boron free, lead barium silicate glasses of this invention is highly positive. Such a TCR effect can be neutralized by the addition to the system of a metal oxide which has a highly negative TCR. Examples of such metal oxides include, SnO<sub>2</sub>, Cr<sub>2</sub>O<sub>3</sub>, Bi<sub>2</sub>O<sub>3</sub>, and TiO<sub>2</sub>. Preferred for the purposes of

this invention is MnO<sub>2</sub> which is highly negative and thus need be employed in only small amounts.

The amounts of each ingredient employed in the resistor compositions of this invention will vary over a wide range depending upon the various characteristics desired in the ultimate product, the various sub-systems and metals etc. employed and the like. Generally speaking, the preferred use for the resistor compositions of this invention is in the microelectronic printed resistor art wherein a microelectronic resistor pattern in paste form is first printed in a desired pattern and then fired to its ultimate structure. The resistors so formed preferably exhibit a stability factor of less than about  $\pm 1\%$  drift during normal load life (e.g. 10 1000-10,000 hrs.) and have a TCR of less than  $\pm 500$  ppm/°C, preferably less than  $\pm 200$  ppm/°C and most preferably about  $\pm 0$  ppm/°C (i.e. less than about 100 ppm/°C), measured at 25°-150°C. In the most preferred embodiments the above characteristics of an individual resistor system are reproducible usually on the order of about  $\pm 20\%$  or less.

In the achievement of the above, the metal content of the metal powder should be comprised by weight percent of about 5-95% by weight of the resistive metal system, preferably palladium alone, and preferably in amounts of about 15-75% and, most preferably about 20-65%. The remainder of the metal content usually consists of the stabilizer metal system, in weight ratios as described, to minimize effect on TCR.

30 In those instances where an anti-agglomerating agent is employed, it is usually employed in amounts of about 0.5-15% by weight of the total metal powder. In a PdO system, for example where the stabilizer system in an admixture of silver and gold, it is preferred to use a finely divided silica (submicron particle size) anti-agglomerating agent in an amount of about 5% by weight of the total metal powder composition.

The amount of glass binder employed with the above-described powder and the amount of TCR neutralizing oxide will usually depend upon the desired resistivity of the final product and the degree to which its TCR must be reduced toward zero. In those instances where the above-described preferred systems are employed, the general range of constituents for the resistor composition includes by weight about 40-95% glass binder and 5-60% metal powder. In those instances where a TCR neutralizing oxide such as MnO<sub>2</sub> is employed it, usually is employed in relatively low amounts such as, for example, about 0.02-0.5% of the metal powder. In those instances where low resistivities on the order of about 1-400 ohms is desired in the final product, the resistor composition preferably comprises by weight about: 45-55% glass binder and 55-45% metal powder. For higher resistivities greater than 400 ohms and generally about 400-20,000 ohms, the composition preferably comprises by weight about: 50-85% glass binder and 15-50% metal powder.

60 The above-described resistor compositions of this invention may be formulated by intimately blending particles of glass binder, usually less than about 5 microns in size with the metal powder. This may be accomplished by any conventional means such as by comminution and ball milling. Best results are achieved with as high a dispersion degree or blending as is reasonably possible. In those instances where a TCR neutralizing oxide is employed, it is usually added in small particle form (i.e. less than about 5 microns) to the particulate

glass and powder prior to the blending operation so that it too becomes intimately dispersed throughout the composition.

It has been quite unexpectedly found that the unoxidized resistor compositions of this invention, particularly where the metal powder consists of less than about 50% by weight of the resistive metal system, are relatively insensitive, in and of themselves, to oxidation during normal firing processes for microelectronic resistors. For example, the formation of a resistor from paste form using the unoxidized composition usually results in a resistivity of only a few ohms. This is particularly true when the preferred glass binders of this invention are employed such that firing is conducted at about 725°-775°C. Thus comminution, care not to disturb the oxidized structure prior to firing and the like, do not play as large a role in the achievement of reproducibility and insensitivity to firing process fluctuations as they did in the aforementioned U.S. Pat. No. 3,681,261, or in the prior art referred to therein. For this reason several alternatives are available for controlling, with good reproducibility, the amount of resistivity obtained. Firstly, oxidation of the resistive metal in the metal powder may be carried out either before or after the powder is blended with the glass binder. Preferably, oxidation is carried out after initial blending but prior to ball milling, if such is employed, in order to prevent agglomeration problems. Oxidation is effected by conventional techniques, usually by heating the composition in air to a temperature high enough to effect oxidation, but not high enough to retard it. Such temperatures are usually on the order of about 300°-650°C. Temperatures which will cause the flow of the glass binder or cause it to sinter should not be employed. Generally, for the preferred glass binders of this invention, oxidation is carried out below about 500°C to avoid any problem of flow or sintering.

One alternative for controlling resistivities is to effect only that degree of oxidation necessary to achieve the desired resistivity. Since the remaining unoxidized composition is relatively insensitive to fluctuations in the firing process, resistivity will usually only change less than a few ohms during firing. Generally speaking, substantially complete oxidation is obtained for most systems of this invention when the systems are heated in air for about 4-16 hours at 300°-650°C. Thus, simple trial and error at shorter times will lead to a specific set of operating conditions to obtain a particular resistivity for each individual system.

A second alternative is to oxidize a resistive composition completely and then blend into it, either before or during printing paste formation, a prescribed amount of unoxidized composition to obtain the desired resistivity. Again, simple trial and error will dictate specific blends for each system. Since the unoxidized composition is generally insensitive in and of itself to firing fluctuations, resistivity will not change to any meaningful extent due to variations in firing temperatures, etc., during firing.

A third alternative is, to combine the first two alternatives described above. Of these three alternatives, the second one is preferred as it is most convenient, easy to regulate, and less subject to fluctuations and variations that may occur during the oxidation step.

The above-described resistor compositions may be employed in a wide variety of ways and environments for their resistive properties. Any of these ways and en-

vironments, conventional in the art, are contemplated by this invention. As alluded to hereinabove, a preferred way in which these resistor compositions may be used is to formulate them into printing pastes and print them on appropriate substrates for use in microelectronic circuitry.

Printing pastes contemplated by this invention comprise an organic liquid vehicle in which the resistor composition is dispersed. Any of the conventional organic liquid vehicles may be employed. A particularly preferred vehicle for the purposes of this invention is a mixture comprised of 85% by weight of a mixture of 2 parts by weight butyl carbitol acetate (diethylene glycol monobutyl ether acetate) to 1 part by weight iso-amyl salicylate and 15% by weight of ethyl cellulose. The amount of vehicle to composition employed will vary over a wide range depending upon the physical dimensions and characteristics of the ultimate resistor desired. Generally speaking, the resistor composition is employed in an amount of about 5-2 parts by weight to 1 part by weight vehicle.

The paste is formed by thoroughly blending the particulate resistor composition with the vehicle by mixing and roller milling. The paste so formed may then be printed in a desired pattern using a conventional screen or mask. Thereafter, the printed design is dried and fired to produce the final resistor, usually upon a dielectric substrate. Drying after printing may be effected by either air drying and/or oven drying, usually at a temperature of about 100°-125°C for about 5-10 minutes. Firing is usually accomplished thereafter at the temperatures indicated above (e.g. 650°-775°C) using a heat-up, peak, and cooldown cycle of about 20-60 minutes with firing at peak temperatures for about 2-15 minutes.

As stated hereinabove, the resulting printed resistors of this invention are found to be highly reproducible, have excellent stability, and generally have TCR's less than  $\pm 500$  ppm/°C, usually less than  $\pm 200$  ppm/°C, and in some instances, substantially close to 0 ppm/°C.

The following examples are presented as illustrative of this invention:

#### EXAMPLES 1-13

45 Resistors were formulated from the following ingredients and by the following process:

A homogeneous palladium, silver, gold metal powder consisting of by weight 35% Pd, 52% Ag and 13% Au, which was substantially free of any silver chloride or cyanide was formulated according to Example 2 of the aforementioned U.S. Pat. No. 3,717,453. X-ray analysis indicated that the Pd and Ag were alloyed while the Au was merely dispersed. The particle size of the powder was in the submicron range. A particulate glass binder consisting of, by weight, 59% PbO, 31% SiO<sub>2</sub>, 2% Bi<sub>2</sub>O<sub>3</sub>, and 8% BaO was blended by mixing into the metal powder and ball milling was employed after oxidation.

60 Oxidation in air was carried out at the indicated time and temperature where indicated. In those examples which indicate the use of MnO<sub>2</sub> (particle size less than 5 microns), this was blended simultaneously with the glass binder into the metal powder. The blends were formulated into pastes by admixing 3 parts by weight solids with 1.1 parts by weight of a liquid organic vehicle consisting of 85% by weight of 2 parts by weight butyl carbitol acetate to 1 part by weight iso-amyl salic-

ylate and 15% by weight of N-4 ethyl cellulose. The pastes were then printed upon 1 inch square alumina substrates using a 200 mesh stencil screen. The printed design was then dried at about 100°C for about 5 minutes and then fired in an open air, continuous, belt conveyor kiln which allowed for a 30 minute firing cycle with 7 minutes at peak. Three designs for each example were formed. They are as follows:

| Design Reference | Dimensions in Mils |        |       |
|------------------|--------------------|--------|-------|
|                  | Width              | Length | Thick |
| Small            | 40                 | 40     | 0.7   |
| Medium           | 80                 | 80     | 0.7   |
| Large            | 200                | 200    | 0.7   |

The following results were obtained using conventional measuring techniques. Resistance was measured by a conventional digital ohmmeter. TCR was measured by measuring resistance at room tem. (25°C), then heating the resistor to 150°C and again measuring resistance. TCR is then calculated by taking the resistance change in ohms times 10<sup>6</sup> divided by the resistance at 25°C times 125°C. This is represented by the formula TCR =  $(\Delta R \times 10^6) / (R_{25^\circ C} \times 125^\circ C)$

## EXAMPLE 14

Example 1 was reconduted except that the gold powder employed in making up the metal powder was commercially obtained from Englehard Industries and had an average particle size of about 1-2 microns. The results were as follows:

TABLE B

| Firing Temp. | Resistance (ohms/sq.) |      |       | TCR (ppm/°C) |      |       |
|--------------|-----------------------|------|-------|--------------|------|-------|
|              | Small                 | Med. | Large | Small        | Med. | Large |
| 725          | 336                   | 372  | 467   | +84          | +73  | +68   |
| 750          | 394                   | 489  | 593   | +90          | +88  | +84   |
| 775          | 391                   | 484  | 722   | +57          | +68  | +61   |

In addition to showing the flexibility of this invention in being able to use various starting materials, the example, compared with example 1, shows the reproducible nature of the resistors of this invention.

Once given the above disclosure, many other fea-

TABLE A

| No. Formulation<br>(Metal/glass/<br>MnO <sub>2</sub> wt. ratio) | Firing<br>Temp. °C | Resistance (ohms/sq.) |       |       | TCR (ppm/°C) |      |       | Ox.<br>Time/<br>Temp. | Ball<br>Mill |
|-----------------------------------------------------------------|--------------------|-----------------------|-------|-------|--------------|------|-------|-----------------------|--------------|
|                                                                 |                    | Small                 | Med.  | Large | Small        | Med. | Large |                       |              |
| 1. 10/10/.009                                                   | 725                | 390                   | 450   | 510   | -36          | -33  | -33   | 400°C                 | 24 hrs.      |
|                                                                 | 750                | 400                   | 475   | 540   | -65          | -67  | -57   | 4 hrs.                | 24 hrs.      |
|                                                                 | 775                | 430                   | 550   | 640   | -81          | -76  | -72   |                       | 24 hrs.      |
| 2. 10/10/.008                                                   | 725                | 220                   | 236   | 284   | +140         | +156 | +157  |                       |              |
|                                                                 | 750                | 331                   | 363   | 463   | +117         | +129 | +130  | 4 hrs.                |              |
|                                                                 | 775                | 410                   | 489   | 617   | +115         | +122 | +130  | 400°C                 | 16 hrs.      |
| 3. 10/20/.008                                                   | 725                | 1250                  | 1250  | 1400  | +152         | +157 | +165  |                       |              |
|                                                                 | 750                | 1800                  | 1900  | 2400  | +125         | +142 | +138  | do.                   |              |
|                                                                 | 775                | 2500                  | 3200  | 4000  | +114         | +121 | +127  |                       |              |
| 4. 10/10/.009                                                   | 725                | 1.4                   | 1.6   | 2.1   | —            | —    | —     | N                     |              |
|                                                                 | 750                | .8                    | .9    | 1.1   | —            | —    | —     | O                     |              |
|                                                                 | 775                | 1.1                   | 1.2   | 1.6   | —            | —    | —     | N                     | 16 hrs.      |
| 5. 10/10/.0080                                                  | 725                | 317                   | 337   | 407   | +61          | +59  | +61   | 16 hrs.               |              |
|                                                                 | 750                | 423                   | 500   | 634   | +40          | +48  | +53   | 400°C                 |              |
|                                                                 | 775                | 517                   | 596   | 797   | +50          | +47  | +39   |                       |              |
| 6. Blend-30% No. 4<br>- 70% No. 5<br>(Wt. %)                    | 725                | 170                   | 198   | 257   | +28          | +20  | +16   | —                     | —            |
|                                                                 | 750                | 132                   | 152   | 222   | 0            | -5   | +10   | —                     | —            |
|                                                                 | 775                | 275                   | 274   | 412   | -5           | 0    | -10   | —                     | —            |
| 7. Blend-10% No. 4<br>- 90% No. 5<br>(Wt. %)                    | 725                | 262                   | 292   | 351   | +34          | +42  | +45   | —                     | —            |
|                                                                 | 750                | 269                   | 300   | 385   | +55          | +44  | +45   | —                     | —            |
|                                                                 | 775                | 481                   | 525   | 631   | +39          | +35  | +33   | —                     | —            |
| 8. 1/1/0                                                        | 725                | 65                    | 70    | 95    | +482         | +499 | +518  | 4 hrs.                |              |
|                                                                 | 750                | 65                    | 62    | 75    | +516         | +397 | +541  | 400°C                 | None         |
|                                                                 | 775                | 45                    | 45    | 65    | +473         | +456 | +497  |                       |              |
| 9. 20/80/0                                                      | 725                | >10M                  | >10M  | >10M  | —            | —    | —     |                       |              |
|                                                                 | 750                | 50K                   | 70K   | 80K   | +452         | +433 | +415  | 4 hrs.                |              |
|                                                                 | 775                | 16K                   | 18K   | 18K   | +560         | +560 | +600  | 450°C                 |              |
| 10. 20/80/.0085                                                 | 725                | —                     | —     | —     | —            | —    | —     | 400°C                 |              |
|                                                                 | 750                | 8.8K                  | 11.9K | 15.2K | +284         | +279 | +280  | 4 hrs.                |              |
|                                                                 | 775                | 5K                    | 6.2K  | 7.7K  | +246         | +244 | +248  |                       |              |
| 11. Blend-30% No. 1<br>70%<br>(wt. %)                           | 725                | 2.1K                  | 2.4K  | 2.7K  | +82          | +89  | +90   | —                     | —            |
|                                                                 | 750                | 2.85K                 | 3.4K  | 3.86K | +87          | +76  | +90   | —                     | —            |
|                                                                 | 775                | 3.87K                 | 4.43K | 4.76K | +97          | +63  | +63   | —                     | —            |
| 12. Blend-70% No. 1<br>30% No. 3<br>(wt. %)                     | 725                | 1.21K                 | 1.45K | 1.6K  | +64          | +75  | +76   | —                     | —            |
|                                                                 | 750                | 1.75K                 | 1.9K  | 2.1K  | +66          | +75  | +80   | —                     | —            |
|                                                                 | 775                | 2.3K                  | 2.8K  | 3.0K  | +47          | +45  | +50   | —                     | —            |
| 13. Same as<br>Ex. 3 except<br>oxidized for<br>16 hrs./400°C    | 725                | 1.76K                 | 1.99K | 2.47K | +126         | +121 | +129  | 16 hrs.               |              |
|                                                                 | 750                | 2.68K                 | 3.06K | 3.79K | +113         | +114 | +119  | 400°C                 |              |
|                                                                 | 775                | 3.66K                 | 4.09K | 4.97K | +98          | +102 | +103  |                       |              |

In addition to the above generally excellent electrical properties, the resistors were found to be stable and reproducible as, defined hereinabove.

tures, modifications, and improvements will become apparent to the skilled artisan. Such other features, modifications and improvements are considered to be

a part of this invention, the scope of which is to be determined by the following claims:

I claim:

1. A resistor composition comprising a particulate zinc free, boron free, lead, barium silicate glass binder having a firing temperature of about 725°-775° C. and a positive TCR, said glass binder being admixed with a substantially homogeneous finely divided, substantially chloride or cyanide salt-free powder comprised of at least one resistive metal selected from the group consisting of palladium, rhodium, iridium, ruthenium, indium and mixtures thereof, at least two stabilizer metals selected from the group consisting of silver, gold and platinum, and about 0.02-0.5 weight percent, related to the weight of the metal powder, of particulate MnO<sub>2</sub> to reduce the TCR of said resistor composition.

2. A resistor composition according to claim 1 in which a metal selected from the group consisting of platinum, copper, nickel and mixtures thereof are combined with silver and gold.

3. A resistor composition according to claim 1 having a TCR less than about 200 ppm/°C (25° - 150°C), wherein said resistor composition comprises about 40 - 95 weight percent of a glass binder having a particle size of less than about 5 microns, wherein said glass binder comprises by weight about: 40 - 75% PbO, 15 - 40% SiO<sub>2</sub>, 0 - 15% Bi<sub>2</sub>O<sub>3</sub> and 0 - 15% BaO and wherein about 2 - 30% is Bi<sub>2</sub>O<sub>3</sub> + BaO and the listed oxides constitute at least about 90% by weight of the glass composition, and about 5 - 60% of said metal powder, said MnO<sub>2</sub> having a particle size less than about 5 microns.

4. A resistor composition according to claim 3 wherein said powder also includes about 5 weight percent of a silica having a particle size of less than about 5 microns as an anti-agglomerating agent substantially homogeneously dispersed throughout the powder.

5. A resistor composition according to claim 4 wherein said glass binder consists essentially of by weight about: 59% PbO, 31% SiO<sub>2</sub>, 2% Bi<sub>2</sub>O<sub>3</sub> and 8% BaO.

6. A resistor composition according to claim 5 wherein said powder consists of by weight: 35% Pd, 52% Ag and 13% Au.

7. A resistor composition according to claim 4 having a TCR less than about 100 ppm/°C (25° - 150°C.)

8. A resistor composition according to claim 1 wherein said stabilizer metals are selected from an admixture of the following metals in the indicated weight ratios: Ag:Au, about 4:1-1:4; Pt:Ag, about 8:1-1:8; and Pt:Au, about 8:1-1:8.

9. A resistor composition according to claim 1 wherein said powder also includes an anti-agglomerating agent substantially homogeneously dispersed throughout the powder, said anti-agglomerating agent being a refractory having a particle size less than about 5 microns.

10. A resistor composition according to claim 3 wherein at least one of said resistive metals is alloyed with at least one of said stabilizer metals.

11. A resistor composition according to claim 1

wherein said resistive metal is palladium.

12. A resistor composition according to claim 11 wherein said stabilizer metals are Ag and Au in a weight ratio of about 4:1-1:4.

13. A resistor composition according to claim 12 wherein Ag is alloyed with Pd.

14. A resistor composition according to claim 1 wherein said glass binder comprises by weight about: 40-75% PbO, 15-40% SiO<sub>2</sub>, 0-15% Bi<sub>2</sub>O<sub>3</sub> and 0-15% BaO wherein about 2-30% is Bi<sub>2</sub>O<sub>3</sub> + BaO and the listed oxides constitute at least about 90% by weight of the glass composition.

15. A resistor composition according to claim 14 wherein said glass binder consists essentially of by weight about: 59% PbO, 31% SiO<sub>2</sub>, 2% Bi<sub>2</sub>O<sub>3</sub>, and 8% BaO.

16. A resistor composition according to claim 1 wherein said powder is comprised of by weight about 5-95% of at least one resistive metal and 95-5% by weight of said at least two stabilizer metals.

17. A resistor composition according to claim 16 wherein said resistor metal is palladium in an amount by weight of about 15-75% of said powder.

18. A resistor composition according to claim 17 wherein said palladium is in an amount by weight of about 20-65% of said powder.

19. A resistor composition according to claim 16 wherein said powder also includes an anti-agglomerating agent in an amount by weight of about 0.5-15% of said powder, said anti-agglomerating agent being substantially homogeneously dispersed throughout the powder and said anti-agglomerating agent having a particle size less than about 5 microns.

20. A resistor composition according to claim 19 wherein said anti-agglomerating agent is finely divided silica in an amount by weight of about 5% of said powder.

21. A resistor composition according to claim 33 which comprises by weight about 40 - 95% glass binder and about 5 - 60% metal powder.

22. A resistor composition according to claim 1 wherein said powder was formulated by initially forming a soluble salt solution of at least one resistive metal and silver, adding to said solution a finely divided gold powder having a particle size of less than about 5 microns, forming a slurry of said solution and gold powder, and adding a reducing agent to said slurry to precipitate metallic silver and resistive metal.

23. A resistor composition according to claim 22 wherein said resistive metal is palladium.

24. A printing resistor paste comprised of a liquid organic vehicle and the composition of claim 1.

25. A printing resistor paste according to claim 24 wherein said vehicle consists essentially of diethylene glycol monobutyl ether acetate, iso-amyl salicylate and ethyl cellulose.

26. A printing resistor paste according to claim 25 wherein said resistor composition is in an amount of about 5-2 parts by weight per 1 part by weight of said vehicle.

\* \* \* \* \*

UNITED STATES PATENT AND TRADEMARK OFFICE  
CERTIFICATE OF CORRECTION

PATENT NO. : 3,865,742

DATED : February 11, 1975

INVENTOR(S) : B.Greenstein

It is certified that error appears in the above-identified patent and that said Letters Patent are hereby corrected as shown below:

Col. 3, line 14, delete "this copending application" and insert therefor --U.S.Patent No. 3,717,453--; line 25, delete "of this copending aoplication". Col. 5, line 53, delete "ther" and insert therefor --other--; line 60, delete "by" and insert therefor --be--. Col. 8, line 23, after "vehicle" insert --usually--.

Signed and Sealed this  
Nineteenth Day of April 1977

[SEAL]

Attest:

RUTH C. MASON  
*Attesting Officer*

C. MARSHALL DANN  
*Commissioner of Patents and Trademarks*